

Patented May 29, 1923.

## UNITED STATES PATENT OFFICE.

Nail  
Penetrable  
Concrete

No Drawing.

JOHN E. KLEIST, OF NEW ROCHELLE, NEW YORK.

## NAILING CONCRETE.

Application filed November 14, 1922. Serial No. 600,960.

To all whom it may concern:

Be it known that I, JOHN E. KLEIST, a citizen of the United States, residing at 44 Washington Avenue, New Rochelle, in the county of Westchester and State of New York, have invented a new and useful Improvement in Nailing Concrete, of which the following is a specification.

The invention has to do with nailing concrete, that is to say, Portland cement concrete into which nails can be readily driven and which has heretofore been used mainly as a nailing base for floors and roofs in fireproof building construction. The nailing quality of these concretes is obtained by the incorporation in the mixture of an appropriate proportion of asbestos fiber, the comparatively cheap, very short fiber grades being suitable for this purpose. Sand or an equivalent filler is used as is customary in concrete mixtures, the sand or other materials preferably being fine, as coarse particles interfere with the penetration of the nails. The amount of asbestos fiber used varies somewhat according to the grade, and depends in the main on the purpose to which the concrete is to be put. For example, a nailing concrete for a nailing base for wood floors must be comparatively hard, because of the necessity for high holding power on the nails, eight-penny wrought iron nails being customarily used in this class of work. For roofs, on the other hand, soft copper nails are used as a rule to nail the finished roofings, and consequently the concrete must be softer. This so-called hardness of nailing concrete can be controlled by the amount of asbestos fiber in the mixture, the higher percentage of asbestos fiber producing the softer concrete. Depending upon conditions, the amount of asbestos in these mixtures may vary from about 10% to 30% of the total aggregate weight of the whole mixture prior to the addition of water.

The present invention is based upon the discovery that a much better nailing concrete can be produced by the incorporation of a certain percentage of pulverized slate in the mixture. The nailing concrete obtained with the usual mixtures is porous, and the effect of the pulverized slate is partly to fill the voids so that the strength and the nail-holding power of the concrete are greatly increased without destroying the nailing quality. Nails can be driven into this concrete readily and without crack-

ing, and because of the presence of the pulverized slate, there is materially increased compressive friction, which causes the nails to be held more powerfully than heretofore. From the structural standpoint, also, the value of the material is increased because of the greater density, and the high compressive and tensile strength, particularly compressive strength, resulting from the use of the pulverized slate, in mixtures such as are contemplated.

The increase in structural strength obtained in this way is so marked that it becomes possible to adapt nailing concrete, heretofore generally available only as a nailing base, for the production of structural roof and floor slabs complying fully with building code requirements.

The addition of the pulverized slate also has the important effect of rendering the concrete less absorbent of moisture, or comparatively water-proof. The pulverized slate replaces part of the asbestos in the ordinary mixtures, that is to say, less asbestos is used when the slate is added. Tests also show that the pulverized slate in the concrete has binding qualities, and consequently by using a certain percentage of the slate, it is possible to reduce the quantity of Portland cement employed in the mixture, with a consequent reduction in cost.

The proportion of pulverized slate will necessarily vary in different mixtures and for specific purposes, but generally speaking, a percentage of pulverized slate amounting from about one-third to one-half of the weight of asbestos fiber in the mixture has been found suitable. Tests have shown that the following illustrative mixtures produce excellent results.

## No. 1—For wood floors (nailing base).

|                  | By weight. | By volume. |     |
|------------------|------------|------------|-----|
| Portland cement  | 188 lbs.   | 2 cu. ft.  |     |
| Screened sand    | 720 "      | 8 "        |     |
| Pulverized slate | 25 "       | 1 1/2 "    |     |
| Asbestos fiber   | 75 "       | 1 1/2 "    | 100 |

## No. 2—For roofs (nailing base only).

|                  | By weight. | By volume. |     |
|------------------|------------|------------|-----|
| Portland cement  | 188 lbs.   | 2 cu. ft.  |     |
| Screened sand    | 360 "      | 4 "        |     |
| Pulverized slate | 50 "       | 1 1/2 "    |     |
| Asbestos fiber   | 100 "      | 2 1/2 "    | 105 |

## No. 3—For structural roof slabs (slab and nailing base combined).

|                  | By weight. | By volume. |     |
|------------------|------------|------------|-----|
| Portland cement  | 188 lbs.   | 2 cu. ft.  |     |
| Screened sand    | 360 "      | 4 "        |     |
| Pulverized slate | 25 "       | 1 1/2 "    |     |
| Asbestos fiber   | 75 "       | 1 1/2 "    | 110 |

To meet different conditions it will naturally be necessary to have other mix-

tures. For greater certainty it may be stated that these particular mixtures contemplate a grade of asbestos known commercially as "asbestos sand," which consists practically entirely of asbestos fiber in very short form, but other grades of asbestos or asbestos residue may be used.

For purposes of comparison with the illustrative mixtures Nos. 1 and 2, two mixtures that have commonly been used in the past for the same purpose and composed of the same ingredients, lacking, however, the pulverized slate, are set down:

|        |                  | By weight. | By volume. |
|--------|------------------|------------|------------|
| 15     | For wood floors. |            |            |
|        | Portland cement  | 282 lbs.   | 3 cu. ft.  |
|        | Screened sand    | 630 "      | 7 "        |
|        | Asbestos fiber   | 100 "      | 2½ "       |
|        | For roofs.       |            |            |
|        | Portland cement  | 188 lbs.   | 2 "        |
|        | Screened sand    | 360 "      | 4 "        |
| 20 264 | Asbestos fiber   | 200 "      | 4½ "       |

Mixtures of this character are greatly improved and may be cheapened by the incorporation of the pulverized slate, and in addition, it is possible to employ mixtures such as No. 3 for roof or floor slabs.

In the use of the invention, it will be

found convenient for the manufacturer to provide a mixture of the asbestos fiber and pulverized slate to be shipped in bags to different localities and there combined on the spot with the Portland cement and sand or its equivalent, in accordance with formulae supplied. The concrete is made by mixing the ingredients together and adding water in proper amount to cause the cement to set. The concrete when set and dried out is nailable and always remains so, and possesses the improved and additional characteristics due to the presence of pulverized slate.

What is claimed as new is:

A nailable concrete mixture for structural slabs comprising cement, said, asbestos fiber and pulverized slate in approximate proportions as follows:

|                  |          |            |
|------------------|----------|------------|
| Cement           | 188 lbs. | 2 cu. ft.  |
| Sand             | 360 lbs. | 4 cu. ft.  |
| Asbestos         | 75 lbs.  | 1½ cu. ft. |
| Pulverized slate | 25 lbs.  | ¾ cu. ft.  |

JOHN E. KLEIST.